

## UNITED STATES PATENT OFFICE.

WILLIAM JOSEPH OWENS, OF SAN FRANCISCO, CALIFORNIA.

## ADHESIVE MATERIAL.

No Drawing.

Application filed March 31, 1921. Serial No. 457,464.

*To all whom it may concern:*

Be it known that I, WILLIAM JOSEPH OWENS, a citizen of the United States, and a resident of the city and county of San Francisco and State of California, have invented a new and useful Adhesive Material, of which the following is a specification.

This invention relates to building material and particularly to adhesive material used in the manufacture of sheet-like composition material formed of wood and paper, and suitable for walls, partitions and the like.

It is an object of the present invention to provide an improved composition board that is of highly fire-resistant properties.

It is a further object of the present invention to provide a composition board that is comparatively inexpensive in cost of construction and in cost of materials of which it is composed.

It is further an object of the present invention to provide an improved fire resistant and adhesive substance particularly useful in the construction of composition boards.

The invention possesses other objects and features of advantages, some of which, with the foregoing, will be made manifest in the following description of the preferred form of the invention. It is to be understood that it is not intended to limit the invention to the embodiment set forth in the description as variations may be adopted within the scope of the invention as set forth in the claim.

A well known type of composition board is that which embodies a generally plane body structure, consisting of an arrangement of flat, thin lath set substantially edge to edge and coated on the opposite faces of

the whole with sheets of fiber or chip board adhesively secured to the faces of the lath body.

This invention embodies a composition board characterized by the utilization of a fire resistant adhesive mixture which serves the purpose not only of adhesively securing the outer chip-board or paper to the body of laths but also, by substantially entirely embedding each of the laths, materially increasing the fire resistant properties of the whole construction, so that even if the chip-board or paper be scorched or burned the wooden body or lath of the structure will still be preserved against burning by the enclosing fire resistant adhesive.

A fire resistant adhesive is produced by the following: One quart of white glue is dissolved for twelve hours in one and one-half quarts of water. There is then thoroughly mixed with the dissolved glue, two quarts of finishing plaster, preferably in dry condition, one quart of clingstone magnesite in finely powdered form, and three-quarters of a quart of whiting. This composition is thoroughly mixed and heated to about 150° Fahrenheit and is applied to the lath body while in heated condition to prevent setting of the adhesive before the chip-board is applied.

What is claimed is:

A fire resistant adhesive consisting of a mixture of one part white glue dissolved twelve hours in one and one-half parts water; two parts finishing plaster (dry) one part magnesite, and three-quarters part whiting, all by volume.

In testimony whereof, I have hereunto set my hand.

WILLIAM JOSEPH OWENS.